

July 31, 1956

C. E. DIXON

2,756,513

PROCESS FOR THE DRYING OF TIMBER OR OTHER MATERIALS

Filed Aug. 27, 1952



FIG. 1.



FIG. 2.

INVENTOR

CHARLES EDWIN DIXON

By:

Haseltine, Lake & Co.

AGENTS

1

2,756,513

## PROCESS FOR THE DRYING OF TIMBER OR OTHER MATERIALS

Charles Edwin Dixon, Armadale, Victoria, Australia

Application August 27, 1952, Serial No. 306,668

5 Claims. (Cl. 34—37)

This invention relates to an improved method for drying and reconditioning timber.

One known process for the drying of timber is carried out in a ventilated kiln at relatively low temperatures. Air is circulated through the kiln and heated by various means such as steam pipes. This process is slow in operation and is difficult to operate efficiently.

In more recent modifications of this process, the drying is carried out in a ventilated kiln, but at higher temperatures (up to 240° F.).

In the vapour drying or solvent seasoning process, air is excluded from the kiln as far as possible and solvent (working fluid) is circulated in vapour form at high temperatures. Although this process gives a faster drying rate than the low temperature ventilated kiln type of drying, there are several disadvantages inherent in its use. These are (a) explosion and fire risk due to the nature of the volatile solvent; (b) the solvent being relatively expensive, the operational costs are high and (c) little (if any) flexibility of control as the process is normally carried out at the boiling point of the solvent.

One object of the present invention is to provide a process for the drying of timber which can be carried out more rapidly (and consequently more economically) and with greater simplicity of control than the first-mentioned known process.

A further object is to provide a process which substantially eliminates the fire and explosion risk inherent in the solvent seasoning process and which allows a greater degree of flexibility in the operating conditions than is normally possible in the latter process.

A still further object is to provide a process whereby heat from the products of the process can be effectively utilised.

Another object is to provide a process enabling useful products to be obtained from the drying process much more readily than has heretofore been possible.

Further objects will become apparent from the ensuing description.

According to my invention the material to be dried is dried in and by a completely air-free atmosphere of superheated steam at a temperature of from 240° F. to 400° F. and produced wholly or mainly from the moisture given off from the material being dried. However, live steam produced externally may be sprayed into the drying chamber, or alternatively water may be sprayed on to the heating pipes in the kiln, particularly for the treatment or reconditioning of refractory hardwoods and the removal of "collapse." In this process control of the drying rate is effected by varying the quality of the steam whereas in known processes in which air is not excluded, control is effected by varying the relative humidity.

Normally the kiln will be operated at atmospheric pressure but the process of the invention can be carried out at other pressures if expedient.

The process of my invention is carried out in a non-ventilated air-tight kiln heated by means of flue gases which

2

are passed through fire tubes in the kiln chamber. The gaseous products of the process (effluent) are led off through one or more ducts and may be passed firstly through a heat exchanger to heat broiler-feed water, water 5 to be sprayed on to the fire tubes in the kiln, or for other heating purposes, secondly through a condenser wherein further heat may be extracted and thirdly through a gravity separator in which useful products such as pine oils readily separate from the condensed aqueous medium and may be collected.

To facilitate the detailed description of the preferred form of kiln in which the process of the invention may be carried into practical effect, reference will now be made to the accompanying drawings in which:

Figure 1 is a diagrammatic view of the kiln in side elevation, and

Figure 2 is a sectional plan view of the kiln shown in Figure 1.

The kiln is made preferably of welded sheet metal or galvanised iron stiffened with angle iron or other structural members and is insulated with mineral wool and an outer layer of wood shavings or the like. The inner surfaces of the kiln chamber are coated with an inert preservative material such as phenol-formaldehyde resin or lacquer. The kiln is constructed so as to be an airtight, non-ventilated structure having a safety U-trap and drain (not shown) in the base thereof. The drying chamber 1 in which the wood is stacked for drying is heated by a series of heating coils 3 connected with the flue outlet 8 from a step grate 7 by means of flue 9. The drying chamber 1 is provided with a loading door 2 which opens on to a trench 5 below the level of ground 6. The flue gases after passing through the coils 3, enter a further series of heating coils 13 through header 4 and then 20 pass to the stack 12 through flue 10. The heating coils 3, 13 are arranged to give uniformity of heat transfer throughout the chamber and are disposed below a false floor in the form of a baffle 21 which extends the full length of the drying chamber 1 but is clear from each side wall thereof. A by-pass flue 11 directly connects the outlet flue 8 with the stack 12, the path of the flue gases being controlled by means of a baffle 19 which is mounted for pivotal movements in the flue 10 at the junction of the latter and the by-pass flue 11.

40 An outlet duct 14 leads off from the upper part of the drying chamber 1, passes firstly through a heat exchanger 15 and then leads into a U-type gravity separator having a collecting tank 16 and outlets 17, 18. A pipe 20 from which steam may be sprayed into the drying chamber 1 or from which water may be sprayed onto the heating pipes is also provided.

45 In accordance with the invention, the drying is effected in and by a completely air-free atmosphere of steam which is derived wholly or mainly from the moisture given off by the material being dried and is superheated above the saturation temperature to a degree necessary to give the required drying rate. The range of drying temperatures of the kiln atmosphere varies between the 50 240° F. and 400° F. and is preferably between 300° F. and 400° F. No air is present after the initial air has been expelled from the kiln and from this stage until the 60 temperature rises above 212° F. (at atmospheric pressure) no effective drying takes place. Steam of low "quality" or at saturation may result in the reverse of drying, i. e. the raising of the moisture content of the timber being dried, particularly if the timber is at low 65 moisture content. By raising the "quality" of the steam, drying of the timber may be effected.

70 The temperature of the drying chamber is controlled by operation of baffle 19. If the latter is pivoted to a position whereby the by-pass flue 11 is closed, all the flue

gases will pass from the grate 7 through the heating coils 3, 13 and the full heating effect of the flue gases will be felt in the drying chamber. If, however, the baffle 19 is moved so as to close the flue 10, all the flue gases will pass directly from the grate 7 to the stack 12 and the flue gases will not pass through the heating coils at all. In intermediate positions of the baffle, a portion of the flue gases will pass through the heating chamber and it is obvious that control of the temperature (dry-bulb) in the heating chamber can be controlled by suitable manipulation of the baffle.

By utilising high temperatures—up to 400° F.—advantage can be taken of rapid transfusion of moisture through the wood and of the greater plasticity of wood at such temperatures. By simple control of the dry bulb temperature, any drying rate from zero to the maximum possible for the material can be obtained.

Thus the dry bulb temperature is the controlling factor and the process can be readily controlled to produce optimum drying conditions as required for the particular material being treated. This method of control stands in obvious and favourable contrast to earlier methods wherein the relative humidity of the atmosphere in the kiln controlled the drying rate of the charge. In processes of that type, complicated tables of relative wet and dry bulb temperatures were required for control purposes and a relatively small change in the wet bulb depression often caused a relatively large change in the drying conditions in the kiln. Thus, in the old processes, two temperatures (or one temperature and a wet bulb depression) were necessary to describe the schedule of drying conditions and these temperatures were not related to a "base" temperature. In the present process, however, there is a "base" temperature, namely the saturation temperature (usually 212° approx.) and the particular temperature (dry bulb) containing at any time therefore completely describes the schedule of drying conditions at that time.

The heat of the effluent from the drying chamber may be used conveniently to pre-heat boiler-feed water or for other purposes by means of heat exchanger 15 before the condensate is passed to the gravity separator in which useful products such as pine oils separate from the aqueous medium. The pine oils or similar products will collect on the surface of the condensed liquid in tank 16 and pass off through outlet 17. Outlet 18 drains off aqueous condensate from the other arm of the separator. An extremely simple method of recovering the extractives is thus available. At the same time, the determination of the progress of the drying process can be obtained and derived from the measurement of the effluent from the drying chamber or from the measurement of the out-flow from, and the in-flow into, the drying chamber.

The invention thus enables drying and reconditioning of timber to be carried out more economically than in ventilated kilns or by the solvent seasoning process. The higher drying temperatures of the present process substantially reduce the drying time as compared with treatment in ventilated kilns while there is no loss of expensive solvent as occurs in the vapour seasoning process. The explosion and fire risk of the latter process is also effectively overcome by my method. It is thus obvious that the present invention has many advantages over methods at present in use.

I claim:

1. A method of rapidly drying and reconditioning timber, such drying and reconditioning being carried out at one and the same time, by one and the same process and in one and the same kiln chamber, by heating the said kiln chamber to temperatures from 240° F. to 400° F. in the complete absence of air by means of piped flue gases passed through the said kiln chamber in such manner as to give uniformity of heat transfer throughout the said kiln chamber, the heat thus produced in the said kiln chamber firstly causing water to be evaporated from the kiln charge while air is still present in the said kiln

chamber and until all the air originally present in the said kiln chamber is expelled by the expansion caused by the evaporation of the water from the kiln charge, no further drying then taking place until the temperature in the said kiln chamber has been raised above the boiling point of water at the location of the kiln, at which time the kiln atmosphere, being completely free of air, consists wholly of water vapor or superheated steam and wood extractives, the said water vapour or superheated steam and wood extractives being obtained solely from the kiln charge itself, the system being a completely re-circulatory closed one within the kiln chamber, in which drying and reconditioning take place concurrently, the reconditioning and the rate of drying being controlled by the degree of superheat of the said steam or water vapour as indicated by the dry-bulb temperature alone, the wet-bulb temperature remaining constant at the boiling point of the water, the said dry-bulb temperature being controlled by controlling the flow of the piped flue gases passing through the kiln chamber so that the said drying rate is controlled and the desired schedule is maintained directly and solely by controlling the flow of the said piped flue gases and the determination of the progress of the drying process being obtained and derived from the measurement of the effluent from the said kiln chamber and further comprising exhausting the steam as given off.

2. A method of rapidly drying and reconditioning timber, such drying and reconditioning being carried out at one and the same time, by one and the same process and in one and the same kiln chamber, by heating the said kiln chamber to temperatures from 240° F. to 400° F. in the complete absence of air by means of piped flue gases passed through the said kiln chamber in such manner as to give uniformity of heat transfer throughout the said kiln chamber, the heat thus produced in the said kiln chamber firstly causing water to be evaporated from the kiln charge while air is still present in the said kiln chamber and until all the air originally present in the said kiln chamber is expelled by the expansion caused by the evaporation of the water from the kiln charge, no further drying then taking place until the temperature in the said kiln chamber has been raised above the boiling point of water at the location of the kiln, at which time the kiln atmosphere, being completely free of air, consists mainly of water vapour or super-heated steam and wood extractives obtained from the kiln charge itself, the remainder of the kiln atmosphere comprising water vapour or super-heated steam introduced into the kiln chamber, the system being a completely re-circulatory closed one within the said kiln chamber, in which drying and reconditioning take place concurrently, the reconditioning being controlled partially by the quality of the water vapor or super-heated steam introduced into the said kiln chamber, and the rate of drying being controlled and the reconditioning partially controlled by the degree of super-heat of the kiln atmosphere as indicated by the dry-bulb temperature alone, the wet-bulb temperature remaining constant at the boiling point of the water, the said dry-bulb temperature being controlled by controlling the flow of the piped flue gases passing through the kiln chamber so that the said drying rate is controlled, the reconditioning partially controlled and the desired schedule maintained directly and solely by controlling the flow of the said piped flue gases and the determination of the progress of the drying process being obtained and derived from the measurement of the out-flow from, and the in-flow into, the said kiln chamber and further comprising exhausting the steam as given off.

3. In a method of drying timber according to claim 1, the step of obtaining wood extractives by condensing the vapourised extractives directly from the kiln atmosphere without the use of solvents for the said extractives.

4. A method of rapidly drying and reconditioning timber, such drying and reconditioning being carried out at one and the same time, by one and the same process

and in one and the same kiln chamber, by heating the said kiln chamber to temperatures from 240° F. to 400° F. in the complete absence of air by means of piped flue gases passed through the said kiln chamber in such manner as to give uniformity of heat transfer throughout the said kiln chamber, the heat thus produced in the said kiln chamber firstly causing water to be evaporated from the kiln charge while air is still present in the said kiln chamber and until all the air originally present in the said kiln chamber is expelled by the expansion caused by the evaporation of the water from the kiln charge, no further drying then taking place until the temperature in the said kiln chamber has been raised above the boiling point of water at the location of the kiln, at which time the kiln atmosphere, being completely free of air, consists wholly of water vapour or super-heated steam and wood extractives, the said water vapour or super-heated steam and wood extractives being obtained solely from the kiln charge itself, the system being a completely re-circulatory closed one within the kiln chamber, in which drying and reconditioning take place concurrently, the reconditioning and the rate of drying being controlled by the degree of super-heat of the said steam or water vapour as indicated by the dry-bulb temperature alone, the wet-bulb temperature remaining constant at the boiling point of the water, the said dry-bulb temperature being controlled by controlling the flow of the piped flue gases passing through the kiln chamber so that the said drying rate is controlled and the desired schedule is maintained directly and solely by controlling the flow of the said piped flue gases and the determination of the progress of the drying process being obtained and derived from the measurement of the effluent from the said kiln chamber, the vapourised wood extractives being condensed directly from the kiln atmosphere and collected and further comprising exhausting the steam as given off.

5. A method of rapidly drying and reconditioning timber, such drying and reconditioning being carried out at one and the same time, by one and the same process and in one and the same kiln chamber, by heating the said kiln chamber to temperatures from 240° F. to 400° F. in the complete absence of air by means of piped flue gases passed through the said kiln chamber in such manner as to give uniformity of heat transfer throughout the said kiln chamber, the heat thus produced in the said kiln chamber firstly causing water to be evaporated from the kiln charge while air is still present in the said kiln chamber and until all the air originally present in the said kiln chamber is expelled by the expansion caused by the evaporation of the water from the kiln charge, no fur-

ther drying then taking place until the temperature in the said kiln chamber has been raised above the boiling point of water at the location of the kiln, at which time the kiln atmosphere, being completely free of air, consists mainly of water vapour or super-heated steam and wood extractives obtained from the kiln charge itself, the remainder of the kiln atmosphere comprising water vapour or super-heated steam introduced into the kiln chamber, the system being a completely re-circulatory closed one within the said kiln chamber, in which drying and reconditioning take place concurrently, the reconditioning being controlled partially by the quality of the water vapour or super-heated steam introduced into the said kiln chamber, and the rate of drying being controlled and the reconditioning partially controlled by the degree of super-heat of the kiln atmosphere as indicated by the dry-bulb temperature alone, the wet-bulb temperature remaining constant at the boiling point of the water, the said dry-bulb temperature being controlled by controlling the flow of the piped flue gases passing through the kiln chamber so that the said drying rate is controlled, the reconditioning partially controlled and the desired schedule maintained directly and solely by controlling the flow of the said piped flue gases and the determination of the progress of the drying process being obtained and derived from the measurement of the out-flow from, and the inflow into, the said kiln chamber, the vapourised wood extractives being condensed directly from the kiln atmosphere and collected and further comprising exhausting the steam as given off.

#### References Cited in the file of this patent

#### UNITED STATES PATENTS

|    |           |               |       |               |
|----|-----------|---------------|-------|---------------|
| 35 | 649,758   | Robertson     | ----- | May 15, 1900  |
|    | 1,059,820 | Besemfelder   | ----- | Apr. 22, 1913 |
|    | 1,678,559 | Devine        | ----- | July 24, 1928 |
|    | 2,119,261 | Andrews       | ----- | May 31, 1938  |
|    | 2,127,638 | Brandwood     | ----- | Aug. 23, 1938 |
| 40 | 2,376,612 | Muench et al. | ----- | May 22, 1945  |
|    | 2,446,147 | Walund        | ----- | July 27, 1948 |
|    | 2,548,403 | Smith         | ----- | Apr. 10, 1951 |
|    | 2,618,560 | Leslie        | ----- | Nov. 18, 1952 |

#### OTHER REFERENCES

- Special Methods of Seasoning Wood, High-Temperature Drying. Forest Products Laboratory Report 1665-1. Revised May 1954, 5 pages.
- 50 Special Methods of Seasoning Wood, Superheated Steam. Forest Products Laboratory Report #R1665-1. March 1947, 1 page.